

1

2,776,933

## METHOD OF OXIDIZING ASPHALTS

Henry G. Gossen, Ioco, British Columbia, Canada, assignor to Esso Research and Engineering Company, a corporation of Delaware

No Drawing. Application June 16, 1953,  
Serial No. 362,143

3 Claims. (Cl. 196—74)

The present invention concerns an improved process for air-blowing petroleum asphalts. More particularly, it relates to an improved process for oxidizing residual petroleum stocks by air-blowing them in the presence of ferric chloride. The present improvement relates to the type of ferric chloride employed in the asphalt air-blowing operation and in the manner of adding the ferric chloride to the asphalt. Essentially, the present improvement consists in employing ferric chloride in the form of  $\text{FeCl}_3 \cdot 6\text{H}_2\text{O}$  which has been liquefied by heating it above its congruent melting point. In other words, the

$\text{FeCl}_3 \cdot 6\text{H}_2\text{O}$

is heated to a temperature such that it dissolves in its own water of crystallization, and the resulting solution is then added to an asphalt that is being oxidized by a conventional air-blowing process.

The production of oxidized asphalts by blowing air through a petroleum residue or straight run asphalt at elevated temperatures is well known in the art of petroleum refining. It has been established that such a procedure has a decided effect upon the physical properties of the asphalt. In general, this technique serves to increase the hardness, softening point, pliability, and weathering resistance of an asphalt and decreases its ductility and susceptibility to changes in temperature. It will be noted that the hardness of a straight run asphalt may be greatly increased by extensive steam or vacuum distillation of the asphalt, but the resulting product in this instance is generally very temperature susceptible. The air-blowing technique, in comparison with the vacuum distillation method, is capable of producing an asphaltic product of greater pliability but of the same hardness as an asphaltic product produced by vacuum distillation of the same straight run asphalt. As a result of their very desirable hardness, pliability and weathering resistance qualities, oxidized asphalts have become very popular in the production of roofing asphalts, protective coatings, electrical insulating compositions, moulded articles, and the like. In general, oxidized asphalts are available having softening points of about 100° F. to 250° F. or more and penetrations of about 200 down to about 10 (100 g./5 sec./77° F.). By comparison, straight reduced asphalts are generally available possessing softening points of about 100° F. to 170° F. and having penetration values of about 200 down to 10 or 20 (100 g./5 sec./77° F.).

In connection with the conventional process of air-blowing petroleum asphalts, it has further been found that certain materials may be added to the asphalt being processed which will further modify the physical properties of the final product. For example, it has been established that compounds such as ferric chloride make possible the production of air-blown asphalts having even greater softening points for a given penetration than is possible by air-blowing alone. The use of these materials also greatly reduces the period of time usually required in an air-blowing operation.

2

Up to the present time, it has been conventional practice in an asphalt air-blowing operation to add solid ferric chloride to an asphalt for the purpose of catalyzing the reaction and also for controlling the properties of the final product. It has further been found that solid  $\text{FeCl}_3 \cdot 6\text{H}_2\text{O}$  appears to be somewhat superior to other solid forms of ferric chloride in such an operation. This technique, while it is superior to the use of air alone, still possesses certain disadvantages. It has been observed that considerable foaming generally occurs when the solid ferric chloride employed contains any water of crystallization. Furthermore, it has generally been difficult to achieve good mixing of the solid ferric chloride with the asphalt with the result that its catalytic effectiveness has not been completely utilized. In addition, the use of any form of ferric chloride adds to the cost of the final product, thus making it desirable to find a method for reducing the amount of this material required for an air-blowing operation.

Accordingly, it is an object of the present invention to provide a method for rapidly and efficiently dispersing ferric chloride throughout an asphalt without undesirable foaming. It is an additional object of the present invention to provide a means for more conveniently handling (storing and pumping) the ferric chloride prior to its introduction within the asphalt. It is also an object of the present invention to use greatly reduced amounts of ferric chloride in asphalt-blowing operations and yet produce oxidized asphalts possessing substantially the same penetration-softening point relationships as are now provided by larger amounts of ferric chloride.

These and other objects of the present invention may be achieved by (1) using ferric chloride in the form of  $\text{FeCl}_3 \cdot 6\text{H}_2\text{O}$  which is conventionally and commercially available in solid form; (2) by heating the solid

$\text{FeCl}_3 \cdot 6\text{H}_2\text{O}$

to a temperature sufficient to cause its solution in its water of crystallization; and (3) by introducing the resulting liquefied ferric chloride as such within an asphalt in an air-blowing process. It has been discovered that this technique not only reduces the foaming that is normally caused by the addition of solid  $\text{FeCl}_3 \cdot 6\text{H}_2\text{O}$  to a hot asphalt, but also greatly enhances the effectiveness of the ferric chloride in catalyzing the oxidation of the asphalt. For example, it has been established that the amount of  $\text{FeCl}_3 \cdot 6\text{H}_2\text{O}$  required by following this procedure is about  $\frac{1}{4}$  or less than the amount required by adding ferric chloride in solid form. It has also been found that when the  $\text{FeCl}_3 \cdot 6\text{H}_2\text{O}$  is heated to a temperature above 98° F., the  $\text{FeCl}_3 \cdot 6\text{H}_2\text{O}$  dissolves in its own water of crystallization and will remain fluid down to a temperature of about 75° F.—80° F. This feature of the present invention makes it possible to store and pump this material in the form of a liquid rather than as a solid. The benefits derived from this feature are well recognized in the art.

In order to better describe the present invention, it is felt necessary to first briefly describe a conventional process for air-blowing a petroleum asphalt. Generally speaking, a straight-run petroleum asphalt stock having the following physical characteristics is suitable for the production of an oxidized asphalt. It must be free from wax at a low softening point. The asphalt stock must be of a mixed base or naphthenic type. After oxidation it should have a high penetration for a given softening point. It must be ductile and pliable and resistant to weathering.

The asphalt is heated to a temperature of about 400° to not over 520° F. and is passed to a reaction zone

or vessel where it is contacted with streams of air that are generally blown up through the asphalt at rates of about 30 to 60 cu. ft. per min. per ton of asphalt charge. This air-blowing operation is continued until the asphalt charge has reached a desired degree of hardness, penetration, etc. Periods of about 48 to 72 hours are generally required for this purpose when processing 850 barrel batches in horizontal stills. In addition, this process may be carried out either batchwise or continuously, depending upon the equipment available.

Following the air-blowing operation, the oxidized asphalt is removed from the air-blowing zone or reactor and is pumped to any desired location. In some instances,

Portions of a straight run asphalt were oxidized under substantially identical conditions of air rate, temperature, asphalt charge, etc. (1) in the absence of ferric chloride, (2) in the presence of liquefied  $\text{FeCl}_3 \cdot 6\text{H}_2\text{O}$ , (3) in the presence of solid  $\text{FeCl}_3 \cdot 6\text{H}_2\text{O}$  and (4) in the presence of solid  $\text{FeCl}_3$ . It will be appreciated that the hydrates involved did not necessarily exist as the hydrates after 10 they were added to the asphalt. Each portion of asphalt was oxidized to three levels of softening point, and the penetration of the products measured in each instance. The results of this study are shown below.

Table 1

| Asphalt Inspection              | Straight Run Asphalt |     |     | 0.25% $\text{FeCl}_3 \cdot 6\text{H}_2\text{O}$ added as a liquid |     |     | 1% $\text{FeCl}_3 \cdot 6\text{H}_2\text{O}$ added as a solid |     |     | 1% $\text{FeCl}_3$ added as a solid |     |     |
|---------------------------------|----------------------|-----|-----|-------------------------------------------------------------------|-----|-----|---------------------------------------------------------------|-----|-----|-------------------------------------|-----|-----|
| Penetration, 100 g./5 sec./77°F | 38                   | 18  | 12  | 60                                                                | 33  | 25  | 70                                                            | 35  | 27  | 55                                  | 30  | 23  |
| Softening Point, °F             | 140                  | 170 | 200 | 140                                                               | 170 | 200 | 140                                                           | 170 | 200 | 140                                 | 170 | 200 |

it may be cut back with diluents such as petroleum naphtha, kerosene, fuel oil, etc. The preparation of cut-back asphalts is well known in the art, and it is felt that a detailed description of such an operation is therefore not required here.

When ferric chloride has been added in the past to an asphalt passing through an air-blowing process, the ferric chloride has been conventionally added in the form of a solid to the asphalt directly within the oxidizing zone. Nothing other than the turbulent condition normally existing within an oxidizing zone has been relied upon to disperse the ferric chloride throughout the reaction mixture.

The present invention modifies the process just described in that liquid  $\text{FeCl}_3 \cdot 6\text{H}_2\text{O}$  is the particular form of ferric chloride to be employed. As stated earlier, this hydrate is commercially and conventionally available in solid form. In accordance with the present process, this hydrate is heated to a temperature above 98°F. whereupon the ferric chloride dissolves in its own water of crystallization. This phase of the present process may be carried out in any conventional corrosion-resistant type of vessel such as a steam heated autoclave, electrically heated vessel, or the like.

Once liquefied, the ferric chloride may be stored in conventional corrosion-resistant storage tanks in liquid form down to temperatures of about 70°-80°F.

The ferric chloride solution may be added to the hot asphalt either within the reactor or within the transfer line through which the asphalt flows to the reactor. It is preferred that the ferric chloride be added to the asphalt within the transfer line but either method may be used. Better contact and mixing is generally obtained by addition of the catalyst to the transfer line. Usually 1% or less by weight is all the catalyst that need be added. The liquid ferric chloride is preferably added at its ambient temperature (80°-100°F.) by pumping it into the transfer line as charging of the reactor progresses and at a rate calculated to obtain uniform mixing. Agitation may additionally be obtained by air-blowing. Blowing time may vary somewhat, depending upon the nature of the asphalt stock, the design of the apparatus, the relationship of penetration and softening point desired, etc.

The following example serves to better describe the present process and to illustrate the benefits that are derived therefrom.

As demonstrated in the table above, the use of ferric chloride makes possible the production of oxidized asphalts that are beyond the reach of the straight air-blowing process. In addition, the table clearly brings out the ability of the present process to utilize very much smaller amounts of ferric chloride than are conventionally required under substantially identical reaction conditions. In other words, the effectiveness of the ferric chloride is greatly increased.

It will be appreciated that the present process may be modified in various respects without departing from the scope or spirit of the invention. For example, asphalts derived from cracking operations may be processed in a manner similar to straight-run asphalts. In addition, the present oxidation process may be combined with distillation steps to produce asphalts of a wide combination of properties, or residues that have been distilled further than desired may be blended with heavy petroleum distillates before oxidation.

## What is claimed is:

1. In the oxidation of a petroleum asphalt by blowing the asphalt with air in the presence of ferric chloride, the improvement which comprises extraneously liquefying  $\text{FeCl}_3 \cdot 6\text{H}_2\text{O}$  by heating it above its congruent melting point and adding up to about 1 weight percent of the resulting liquid to the asphalt being oxidized.
2. In a process for preparing an oxidized asphalt wherein the asphalt is transported through a conduit to a contacting zone and wherein the asphalt is then contacted with air in the presence of ferric chloride in a conventional manner, the improvement which comprises extraneously melting  $\text{FeCl}_3 \cdot 6\text{H}_2\text{O}$  and incorporating within said asphalt less than about 1.0% by weight of said melted  $\text{FeCl}_3 \cdot 6\text{H}_2\text{O}$ .
3. Process as defined in claim 2 in which the  $\text{FeCl}_3 \cdot 6\text{H}_2\text{O}$  is introduced within the asphalt as it is transported through the conduit.

## References Cited in the file of this patent

## UNITED STATES PATENTS

- 1,782,186 Abson \_\_\_\_\_ Nov. 18, 1930  
2,627,498 Fink et al. \_\_\_\_\_ Feb. 3, 1953

## OTHER REFERENCES

- "Properties of Asphaltic Bitumen" (Pfeiffer), Elsevier Publ. Co., New York, N. Y. (1950), pages 140-141 relied on.